

3,522,109

**PROCESSES FOR PRODUCING DECORATIVE AND  
PROTECTIVE COATINGS ON COPPER METAL**  
Milton E. Wadsworth, Salt Lake City, Utah (% The Ford  
Foundation, P.O. Box 776, Manila, Philippines), and  
Charles K. Hanson, 1609 West 4th North, Salt Lake  
City, Utah 84116

No Drawing. Continuation-in-part of application Ser. No.  
554,340, June 1, 1966. This application Feb. 5, 1969,  
Ser. No. 796,884

Int. Cl. C23f 7/02, 7/00

U.S. Cl. 148—6.14

11 Claims

**ABSTRACT OF THE DISCLOSURE**

A process of imparting ornamental and protective coatings on copper and copper alloys in relatively short intervals of time. The copper or copper alloy is treated with sulfuric or hydrochloric acid at an elevated temperature and under pressure for 15 minutes to 24 hours to form a coating containing copper compounds.

This application is a continuation-in-part of U.S. patent application Ser. No. 554,340, filed June 1, 1966, now abandoned.

It is a primary object of this invention to provide novel processes for coating the exposed surfaces of copper metal, including copper alloys, with an ornamental and protective pigmented layer containing one or more copper compounds.

Another object is to form a coating comprising at least one copper compound upon copper metal by submerging the copper metal and alloys within a solution of controlled reagent concentration and/or pH under conditions of elevated temperature and pressure, preferably achieved by an overpressure of oxygen.

To form a coating layer comprising brochantite,  $\text{CuSO}_4 \cdot 3\text{Cu}(\text{OH})_2$ , or tenorite,  $\text{CuO}$ , upon copper metal, in pure or alloy form, the copper is submerged in an aqueous acid solution of controlled concentration and pH, preferably containing either singly or in combinations of one or more of the following compounds: sulfuric acid, sodium sulfate, sodium bisulfate, and copper sulfate. The solution is heated to a selected suitable temperature for a predetermined time interval and is also subjected to an overpressure of oxygen, preferably within the general range of 30 to 250 p.s.i. The overpressure of oxygen not only appropriately pressurizes the system, but uniquely supplies an oxidizing agent which is helpful in formation of the coating.

The texture, color and/or general appearance of coatings comprising brochantite and tenorite may be varied by subjecting copper metal to different combinations and concentrations of reagents, temperatures, and pressures for various time intervals. It is postulated that a thin film of cuprite is usually formed upon the exposed surfaces of the copper metal over the top of which the brochantite is formed.

To form a coating of atacamite, basic copper chloride, upon copper metal, in pure or alloy form, the copper is submerged in an aqueous acid solution of hydrochloric acid of controlled concentration and pH. The solution is heated to a selected suitable temperature within the range of 90° C. to 95° C. for a predetermined time interval and is also subjected to an overpressure of oxygen, preferably within the general range of 60 p.s.i. to 70 p.s.i. The overpressure of oxygen not only appropriately pressurizes the system, but uniquely supplies an oxidizing agent which is helpful in the formation of the coating.

The time interval for maintaining the desired tempera-

tures in preparing such coatings is determined by the desired thickness of the layer to be produced. It may vary from a fraction of an hour after the desired temperature is reached to many hours, but as much as 24 hours is rarely required. Elevated temperatures are preferably attained through use of an autoclave, which speeds the reaction by which the coatings are produced. Decorative and protective layers are thus formed within a few hours or fraction of an hour in contrast to certain natural patinas which appear only after years of weathering.

By so varying the (a) types, concentrations and pH of the reagent, (b) temperatures, (c) pressures, and (d) time, the color of the coating of brochantite and atacamite can be varied anywhere between emerald green and blackish green. The tenorite so produced is dark black but exhibits superior adherence to the base copper metal.

The results of laboratory testing are set forth below in Table I and Table II, and in Examples 1-4, inclusive.

TABLE I.—pH RELATED TO FILM FORMATION ON COPPER

|      | pH <sub>i</sub> | pH <sub>f</sub> | Temp. | O.P. | $\text{HSO}_4^-$ | $\text{SO}_4^{2-}$ | Time (min.) | Layer                      |
|------|-----------------|-----------------|-------|------|------------------|--------------------|-------------|----------------------------|
| 5.9  | 4.7             | 125             | 125   |      | 0                | 0.5                | 50          | Tenorite.                  |
| 5.1  | 5.2             | 125             | 125   |      | 0                | 1.0                | 45          | Do.                        |
| 4.6  | 4.8             | 125             | 125   |      | 0                | 0.5                | 60          | Tenorite plus Brochantite. |
| 4.2  | 4.3             | 125             | 125   |      | 0                | 0.5                | 60          | Brochantite.               |
| 3.75 | 4.1             | 129             | 125   |      | 0                | 0.5                | 60          | Do.                        |
| 3.4  | 3.5             | 125             | 125   |      | 0                | 0.5                | 30          | Do.                        |
| 3.2  | 3.6             | 125             | 125   |      | 0                | 0.5                | 120         | Do.                        |
| 3.2  | 3.6             | 157             | 1,000 |      | 0                | 0.5                | 30          | Do.                        |
| 3.2  | 3.3             | 125             | 125   |      | 0.001            | 0.1                | 30          | Do.                        |
| 3.2  | 2.7             | 190             | 500   |      | 0.001            | 0.1                | 30          | Do.                        |
| 30   | 3.2             | 165             | 240   |      | 0.001            | 0.1                | 30          | Do.                        |
| 3.2  | 3.2             | 172             | 250   |      | 0.001            | 0.1                | 120         | Do.                        |
| 3.2  | 3.4             | 140             | 150   |      | 0.001            | 0.1                | 1,440       | Do.                        |
| 3.1  | 2.9             | 147             | 1,000 |      | 0.001            | 0.1                | 30          | Do.                        |
| 3.1  | 2.9             | 150             | 230   |      | 0.001            | 0.1                | 30          | Do.                        |
| 3.1  | 3.1             | 125             | 125   |      | 0.01             | 1.0                | 60          | Do.                        |
| 3.0  | 3.3             | 125             | 125   |      | 0                | 0.5                | 60          | Do.                        |
| 35   | 3.0             | 3.1             | 125   | 125  | 0                | 0.1                | 30          | Do.                        |
| 3.0  | 3.2             | 125             | 125   |      | 0.001            | 0.1                | 30          | Do.                        |
| 3.0  | 3.2             | 125             | 125   |      | 0.001            | 0.1                | 30          | Do.                        |
| 2.9  | 3.2             | 125             | 125   |      | 0                | 0.5                | 60          | Cuprite.                   |
| 2.7  | 2.65            | 127             | 125   |      | 0                | 0.5                | 25          | Nothing.                   |
| 40   | 2.5             | 2.7             | 192   | 230  | 0.001            | 0.1                | 105         | Brochantite.               |
| 2.2  | 2.4             | 205             | 250   |      | 0.001            | 0.1                | 30          | Do.                        |
| 1.9  | 2.4             | 130             | 250   |      | 0.001            | 0.1                | 1,260       | Do.                        |
| 1.6  | 2.1             | 205             | 250   |      | 0.001            | 0.1                | 60          | Do.                        |
| 1.6  | 1.7             | 218             | 250   |      | 0.001            | 0.1                | 180         | Nothing.                   |
| 2    | 1.0             | .7              | 125   | 125  | 0                | 0                  | 45          | Do.                        |

<sup>1</sup> 0.01 M  $\text{CuSO}_4$  added.

<sup>2</sup> 0.1 M Sulfuric Acid Only—Where:

(a) pH<sub>i</sub> is the initial pH of the solution.  
(b) pH<sub>f</sub> is the final pH of the solution.  
(c) Temp. is the temperature of the solution in degrees centigrade.  
(d) O.P. is oxygen overpressure in pounds per square inch.  
(e)  $\text{HSO}_4^-$  is the ionic bisulfate molarity added to the solution.  
(f)  $\text{SO}_4^{2-}$  is the ionic sulfate molarity added to the solution.

TABLE II.—pH RELATED TO FILM FORMATION ON COPPER

|    | pH <sub>i</sub> | pH <sub>f</sub> | Temp. | O.P. | HCl   | Time (min.) | Layer      |
|----|-----------------|-----------------|-------|------|-------|-------------|------------|
| 50 | 1.8             | 4.8             | 95    | 60   | 0.016 | 180         | Atacamite. |
|    | 2.0             | 4.4             | 95    | 60   | 0.010 | 180         | Do.        |
|    | 1.8             | 4.4             | 95    | 70   | 0.016 | 180         | Do.        |
| 55 | 2.0             | 3.9             | 95    | 70   | 0.010 | 180         | Do.        |
|    | 2.0             | 3.8             | 95    | 70   | 0.010 | 180         | Do.        |
|    | 1.9             | 5.5             | 90    | 70   | 0.013 | 180         | Do.        |

Where:

(a) pH<sub>i</sub> is the initial pH of the solution.  
(b) pH<sub>f</sub> is the final pH of the solution.  
(c) Temp. is the temperature of the solution in degrees centigrade.  
(d) O.P. is oxygen overpressure in pounds per square inch.  
(e) HCl is the molar concentration of the hydrochloric acid per liter.

**EXAMPLE I**

To coat copper metal with brochantite, using one of the preferred techniques, the copper metal was placed in a bath comprising a 0.5 molar solution of sodium sulfate, the initial pH values of which were adjusted within a suitable range, preferably between 3.0 and 4.8, by addition of sulfuric acid. The temperatures of these solutions were held at about 125° C., while the oxygen overpressures exerted thereon were held at a desired level, preferably between the range of about 125 to 1,000 pounds per square inch.

**3**  
**EXAMPLE II**

Brochantite coatings on copper were also formed using a second preferred technique by submerging the copper in aqueous solution containing 0.1 M sodium sulfate and 0.001 M sodium bisulfate, with the pH adjusted preferably within the interval of 1.6 to 3.4 by addition of sulfuric acid. These solutions were heated to a selected temperature between about 140° C. and 190° C. and the oxygen overpressures were held at a selected level between about 125 and 1,000 p.s.i.

**EXAMPLE III**

A covering of brochantite was formed on copper submerged in solutions of 0.1 molar sodium sulfate, 0.001 molar sodium bisulfate and 0.01 molar copper sulfate with the pH adjusted within the interval 2.7 to 3.3 by addition of sulfuric acid. Each solution temperature was maintained at a desired level between about 125° C. and 190° C. while the oxygen overpressure was adjusted to a selected value within the range of about 125 to 1,000 p.s.i.

**EXAMPLE IV**

Tenorite coatings were prepared using another preferred technique by placing copper metal in an aqueous solution of 0.5 to 1.0 molar sodium sulfate, with a pH thereof retained within the range of 4.6 to 5.9. The temperature of each solution was held at about 125° C. and the oxygen overpressure was adjusted to about 125 pounds per square inch before heating of the solution began.

The invention may be embodied in other specific forms without departing from the spirit or essential characteristics thereof. The present embodiments are, therefore, to be considered in all respects as illustrative and not restrictive, the scope of the invention being indicated by the appended claims rather than by the foregoing description, and all changes which come within the meaning and range of equivalency of the claims are therefore to be embraced therein.

What is claimed and desired to be secured by United States Letters Patent is:

1. In a process for forming decorative and/or protective coatings comprising copper compounds on copper-containing metals, the steps of:

45 placing the copper-containing metal in an aqueous acid solution comprising either sulfuric acid or hydrochloric acid, subjecting the solution to an elevated temperature within the range of 90° C. to 175° C. for the sulfuric acid solution or 90° C. to 95° C. for the hydrochloric acid solution, imposing an overpressure upon the solution within the range from 30 p.s.i. to 250 p.s.i. for the sulfuric acid solution or 60 p.s.i. to 70 p.s.i. for the hydrochloric acid solution; establishing and retaining the pH of the solution within the acid range not less than 1.6; and removing the metal from the solution after a time interval on the order of within the range of about fifteen minutes to twenty-four hours.

**4**

5 2. In a process of synthesizing pigmented layers containing copper compounds upon the exposed surfaces of copper metal comprising subjecting a heated aqueous solution as defined in claim 1 in which said copper metal has been immersed to an overpressure of oxygen while holding the pH of the solution within the range of about 1.6 to 5.9.

10 3. In a process of reacting an aqueous acid solution with the surface of copper metal as defined in claim 1 to create an external decorative and protective layer having at least one copper compound upon the exposed surface of the copper metal comprising formulating said acid solution from the group consisting of sulfuric acid, sodium sulfate, sodium bisulfate, and copper sulfate or hydrochloric acid, singly or in combination, and contacting the surface of the copper metal with said acid solution while controlling the pH of the solution, elevating the temperature of the acid solution, and elevating the pressure exerted above the solution.

15 20 4. A process as defined in claim 3 wherein said layer comprises copper sulfate.

5 5. A process as defined in claim 3 wherein said solution comprises about 0.5 M sodium sulfate, the pH of the solution falls within the range of about 3.0 to 4.8 and said layer is brochantite.

15 25 6. A process as defined in claim 3 wherein said solution comprises about 0.1 M sodium sulfate and about 0.001 M sodium bisulfate, the pH of the solution falls within the range of about 1.6 to 3.4 and said layer comprises brochantite.

30 7. A process as defined in claim 3 wherein said layer comprises cuprite.

8. A process as defined in claim 3 wherein said layer comprises a copper oxide.

35 9. A process as defined in claim 3 wherein said solution comprises about 0.5 to 1.0 M sodium sulfate, the pH of the solution falls within the range of about 4.6 to 5.9 and said layer comprises tenorite.

10. A process as defined in claim 3 wherein said layer comprises atacamite, basic copper chloride.

40 11. A process as defined in claim 3 wherein a gas comprising oxygen is used to exert said pressure.

**References Cited**

**UNITED STATES PATENTS**

|           |         |               |       |            |
|-----------|---------|---------------|-------|------------|
| 258,082   | 5/1882  | Langhammer    | ----- | 148—6.24   |
| 2,419,915 | 4/1947  | Priest et al. |       |            |
| 3,279,957 | 10/1966 | Fink          | ----- | 148—6.24 X |
| 3,284,249 | 11/1966 | Osborn        | ----- | 148—6.24   |

**FOREIGN PATENTS**

535,614 4/1941 Great Britian.

55 RALPH S. KENDALL, Primary Examiner

U.S. Cl. X.R.

148—6.24